

July 14, 1953

F. E. WILLIAMS

2,645,721

IMAGE INTENSIFICATION APPARATUS

Filed Feb. 16, 1952



Inventor:  
Ferd E. Williams,  
by Paul A. Frank  
His Attorney.

## UNITED STATES PATENT OFFICE

2,645,721

## IMAGE INTENSIFICATION APPARATUS

Ferd E. Williams, Schenectady, N. Y., assignor  
to General Electric Company, a corporation of  
New York

Application February 16, 1952, Serial No. 271,881

16 Claims. (Cl. 250—71)

1

This invention relates to image intensification apparatus and, in particular, to tubes wherein X-ray or gamma ray images are converted into intensified light images by electron optical means.

One of the principal uses of X-rays or gamma rays is found in the study of the internal structure of objects. In such study, the object to be examined is irradiated with X-rays and the transmitted rays are permitted to impinge upon a fluorescent screen or X-ray sensitive phosphor screen whereby a visible light image is formed. The chief difficulty encountered in this employment of X-rays is that of obtaining a visible light image having sufficient intensity and definition to permit adequate observation of the internal structure of the object under examination.

In order to intensify the visible light images produced by X-rays transmitted through an object, it has been proposed heretofore that the light emitted by the fluorescent or X-ray sensitive phosphor be directed to impinge upon a photosensitive surface whereby an electron image corresponding to the light image is emitted from the photosensitive surface. The electron image is then focused by electron optical means on an electron-responsive phosphor screen to produce an intensified light image thereon. This latter image then becomes the final image which is utilized for observation purposes.

The above-described prior art apparatus, while it has produced many satisfactory results, has been found to have an inherent limitation resulting from the low quantum efficiency of known photosensitive materials. Even with the most efficient photosensitive materials, e. g., those of the caesium-antimony type, several light quanta from the X-ray responsive phosphor are required to produce one emitted electron from the photosensitive material. Thus, it is seen that, although the brightness of the final light image produced in the above-described apparatus may be increased to a desired level by increasing the acceleration of the electrons emitted from the photosensitive material, the image definition is restricted by the low quantum efficiency of the photosensitive material.

It is, accordingly, a principal object of the present invention to provide image intensification apparatus capable of producing exceptionally high intensification.

Another object of the present invention is to provide image intensification apparatus capable of producing an exceptionally well-defined final visible image.

2

A further object of the present invention is to provide image intensification apparatus in which no chemically active photosensitive materials are required.

5 It is a still further object of the present invention to provide image intensification apparatus in which the number of electrons utilized to form the final intensified light image is independent of the number of photons of visible light emitted from the X-ray responsive phosphor.

10 It is yet another object of this invention to provide image intensification apparatus in which image de-magnification is avoided.

According to a principal aspect of the invention, 15 there is provided an image intensification tube which comprises an image conversion means spaced from an electron gun which directs a defocused electron beam toward the image conversion means. In progressive order from the side 20 facing the electron gun, the image conversion means includes a photoconductor such as amorphous selenium or cadmium sulphide, a thin transparent conductive element, and an X-ray responsive phosphor such as zinc sulphide activated with silver. Positioned traversing the defocused electron beam between the electron gun and the image conversion means is a fine mesh which is coated on the side facing the image conversion means with an electron-responsive phosphor such as zinc cadmium sulphide. Electrons in the defocused electron beam pass 25 through the voids in the mesh and impinge upon the photoconductor to impart a uniform charge to the surface thereof. X-rays transmitted from 30 an object under observation are directed to strike the X-ray responsive phosphor whereby a visible light image corresponding to the X-ray image is emitted. The light from this image irradiates portions of the photoconductor, and such irradiated portions are discharged through the 35 transparent conductor element. Thus, a charge pattern reversely corresponding to the X-ray image is produced on the surface of the photoconductor facing the electron gun. Electrons 40 arriving thereafter from the electron gun are repelled from the charged portions of the photoconductor and their directions of travel reversed. The reversely traveling electrons impinge upon the electron-responsive phosphor to 45 produce a desired intensified final light image having high definition and brightness.

50 The features of the invention desired to be protected herein are pointed out with particularity in the appended claims. The invention itself, 55 together with further objects and advantages

thereof, may best be understood by reference to the following description, taken in connection with the accompanying drawings, in which Fig. 1 is a schematic sectionalized view of one embodiment of the invention; Fig. 2 is a magnified fragmentary section representation of the image conversion means of Fig. 1; Fig. 3 is a greatly enlarged perspective view of a fragment of the mesh of Fig. 1; and Fig. 4 is a schematic sectionalized view of another embodiment of the invention.

Referring particularly now to Fig. 1, there is shown in schematic fashion image intensification apparatus comprising an evacuable tube 1 having an envelope 2 within which are disposed an image conversion means 3, an electron permeable conductive mesh 4 and an electron gun 5. Image conversion means 3 may be conveniently supported adjacent the end of envelope 2 by a mechanical support (not shown), or attached to the inner surface of tube envelope 2 as shown by actual preparation on the inner surface of envelope 2 or by any suitable means such as an adhesive. Image conversion means 3 is adapted to receive X-rays which have been transmitted through an object under examination and to form on its innermost exposed surface a charge pattern or image which reversely conforms to the image created by the incident X-radiation.

The components of image conversion means 3 are more clearly illustrated in the magnified fragmentary view of Fig. 2. The component shown contiguous with the inner surface of tube envelope 2 is an X-ray responsive phosphor or fluorescent material 6 which is capable of emitting light photons in response to X-radiation incident thereupon. Thus when X-ray responsive phosphor 6 is irradiated through tube envelope 2 with a desired pattern of X-rays, it will fluoresce and form a light image corresponding to the X-ray pattern. X-ray responsive phosphors suitable for such application include zinc sulphide activated with silver, zinc cadmium sulphide activated with silver, calcium tungstate and magnesium tungstate. As illustrated, the X-ray responsive phosphor 6 should be prepared so as to be of quite large particle size, e. g. about 20 microns diameter, and should be deposited with suitable binders such as dilute potassium silicate in a relatively thick layer, e. g. about 100 milligrams per square centimeter in thickness. To avoid feedback excitation, it is preferable that the X-ray responsive phosphor have a predetermined emission spectrum as will be more fully explained hereinafter. Suitable methods of preparing X-ray sensitive phosphors are described in the text entitled "Luminescence of Solids," by H. W. Leverenz, published by John Wiley and Sons in 1950. In this connection, specific attention is directed to chapter 3.

Adjacent the X-ray responsive phosphor 6 is a thin transparent conductive layer or element 7 which has a thickness preferably of the order about 0.01 millimeter to 1 millimeter depending upon its area and the desired resolution of the image conversion means. A suitable transparent conductor of this nature is a conductive glass manufactured by the Pittsburgh Plate Glass Company under the trade-name Nesa. The transparent element may also consist of ordinary glass, e. g., borosilicate glass, which has been treated in a well known manner with stannic chloride to form a conductive surface of stannic oxide. Upon the inner surface of transparent conductive element 7 is deposited a photoconductor 8 which has the

property of being rendered conductive through portions of its cross-section which have been irradiated with visible light. Thus, when the interior surface 9 of photoconductor 8 is sprayed with electrical charge carrying particles such as electrons, the charge upon any portion of the surface 9 may be dissipated by irradiating with visible light a portion of surface 10 which is opposite the selected portion of surface 9. The charges so dissipated are then conducted away through transparent conductive layer 7. Photoconductor 8 is preferably deposited in a layer of from about 1 to 10 microns in thickness and may consist of such materials as cadmium sulfide, zinc sulfide, and amorphous or non-crystallized selenium. Suitable methods for preparing and depositing photoconductor 8 are described in the text entitled "Photoelectricity," published by John Wiley and Sons in 1949 by V. K. Zworykin and E. G. Ramberg. Particular attention is directed to chapter 10 wherein appropriate descriptive material may be found.

Electrons for collection upon the surface 9 of photoconductor 8 may be generated by electron gun 5 which comprises a thermionic cathode, shown in the form of a filament 11, an apertured focusing cup 12 and a cylindrical anode 13, all of which are supported in the manner illustrated by conductive leads introduced into envelope 2 through a suitable seal 13. Filament 11 may be energized by a source of direct current conventionally represented by a battery 14, and focusing cup 12 may be maintained at a positive potential of about 10 volts with respect to filament 11 by means of a battery 15. Anode 13, which includes a washer 16 for the purpose of providing an aperture 17, may be maintained at a positive potential with respect to focusing cup 12 and filament 11 by means of a source of direct voltage conventionally represented by battery 18, one side of which is connected to ground as indicated. The voltage of source 18 should be in the neighborhood of a few hundred volts.

In order that desired image intensification may be obtained according to the invention, the electrons emanating from electron gun 5 must be accelerated to a relatively high velocity. This is accomplished by depositing a conductive film 19 upon a portion of the inner periphery of tube envelope 2 and maintaining this film at a high potential with respect to electron gun 5. High voltage may be imparted to conductive film 19 through a ring-sealed conductive washer 20 which makes contact with conductive film 19 as illustrated. The high voltage, which may be of the order of 10 kilovolts, may be supplied to washer 20 through a conductor 21 connected to a suitable source of direct voltage which is here designated B+. Conductive film 19 may consist of graphite or silver which has been applied in well known ways. In addition to serving as a second anode for accelerating the electrons from gun 5 to a high velocity, conductive film 19 provides an electron lens effect to assure uniform cross-sectional current density in the electron beam indicated by dotted lines 22. Thus, conductive film 19 facilitates the production of a uniform cross-sectional current density beam in which the electron trajectories are approximately parallel to an optical axis 23 as is illustrated by the portions of dotted lines 22 extending to the right of washer 20.

To form a final intensified visible image, an electron-responsive phosphor 24 is deposited upon the side of mesh 4 opposite electron gun 5 as

illustrated in the greatly enlarged perspective view of Fig. 3. Mesh 4 is supported about its periphery by washer 20 and may be attached thereto by any suitable means such as silver solder. As stated hereinbefore, mesh 4 should be quite fine and may consist of a nickel mesh having 400 lines per inch with 50% voids. Such a mesh may be obtained from the Buckbee-Mears Company of St. Paul, Minnesota. The electron-responsive phosphor 24 may be deposited upon mesh 4 by any of the well known methods of spraying, liquid settling, or flotation. A description of such methods may be found in the above-mentioned text entitled "Luminescence of Solids." Phosphor 24 may also be deposited by chemical deposition as described in an article by F. J. Studer, D. A. Cusano, and A. H. Young, appearing in the "Journal of the Optical Society of America," vol. 41, p. 559 (1951). Phosphor 24 preferably consists of zinc cadmium sulphide, or a mixture of zinc sulphide and zinc cadmium sulphide both of which have been activated with silver. Other suitable materials known to those familiar with this art may be employed with efficacy.

In the operation of the apparatus of the invention, the accelerated electrons generated by electron gun 5 form a crossover as indicated at 25 and provide therebeyond defocused electron beam 22. The electrons are further accelerated and constrained into approximately parallel trajectories with respect to optical axis 23 by the potential applied to conductive film 19 whereby an electron beam having substantially uniform cross-sectional current density is produced. A substantial proportion of the accelerated electrons pass through the voids in mesh 4 and proceed to impinge upon the surface 9 of photoconductor 8. In a matter of milliseconds or less, however, surface 9 accumulates enough charge so that electrons arriving at a later time are repelled and caused to return and impinge upon electron-responsive phosphor 24. To assure sufficient collection of charge by surface 9 of photoconductor 8 and also to provide a path for the dissipation of charges from photoconductor 8, a circuit comprising a resistor 26 and a source of direct voltage 27 may be connected to the peripheries of photoconductor 8 and conductive layer 7 through a lead 28 suitably sealed into tube envelope 2. It is pertinent to observe here that the polarity of battery 27 need not always be positive with respect to focusing cup 12. In practice, it has been found preferable to adjust the polarity of battery 27 to produce the best final light image upon phosphor 24, and the voltage required for this purpose has been found to vary between about  $\pm 25$  volts.

After the surface 9 of photoconductor 8 has been charged uniformly by the collection of electrons from beam 22, the irradiation of X-ray responsive phosphor 6 with an X-ray pattern produces a corresponding light image from which photoconductor 8 is irradiated to dissipate charge from corresponding portions of surface 9 through conductive layer 7. As long as light from the X-ray excited phosphor 6 continues to be incident upon portions of photoconductor 8, electrons in beam 22 which arrive at these portions will be collected and dissipated through conductive film 7. Electrons from beam 22 which arrive at non-irradiated portions of photoconductor 8 will continue to be reversed in direction by the charge remaining upon such non-irradiated portions and caused to impinge upon electron-

responsive phosphor 24. In this manner a reverse light image of the object under examination is formed upon electron-responsive phosphor 24. This final intensified light image is viewed through a suitable optical system 29 which may include a condensing lens 28' and a viewing screen 29' positioned exteriorly of envelope 2.

It will not be understood that the final intensified image formed upon electron-responsive phosphor 24 has very high definition. Since the number of electrons generated by electron gun 5 may be increased to any desired amount, an electron beam of very high current density may be produced. When the current density of the electron beam is increased, the number of electrons striking electron-responsive phosphor 24 to form the final visible image is correspondingly increased and hence the definition of the final image may be made very high. Furthermore, it is apparent that the apparatus of Fig. 1 does not utilize any chemically active materials; hence the difficulties of evacuating tube 1 are greatly reduced.

To avoid the possibility that light from the electron-responsive phosphor 24 may irradiate to some extent the photoconductor and result in a deleterious feedback effect, the phosphors and the photoconductor should be selected to have particular emission spectra and a photosensitivity spectrum, respectively. More particularly, the emission spectrum of electron-responsive phosphor 24 should be selected, in conjunction with the photosensitivity spectrum of photoconductor 8, such that light from electron-responsive phosphor 24 does not modify the charge upon photoconductor 8. Similarly, the emission spectrum of the X-ray responsive phosphor should be selected, in conjunction with the photosensitivity spectrum of photoconductor 8, such that light from X-ray responsive phosphor 6 does not modify the charge upon photoconductor 8. These purposes may be effectuated by the use of proper materials. A suitable example is the following: (a) For the X-ray responsive phosphor, hexagonal zinc sulphide activated with silver having a peak emission at 4400 angstroms; for the photoconductor, amorphous red selenium having high sensitivity at 4400 angstroms and negligible sensitivity at 5600 angstroms; for the electron-responsive phosphor, hexagonal zinc cadmium sulphide activated with silver and having a peak emission at about 6000 angstroms. The hexagonal zinc sulphide should be prepared to have a relatively large particle size, e. g. about 20 microns diameter, and should be deposited about 100 milligrams per sq. centimeter thick. The amorphous red selenium should be a few microns thick and is prepared by evaporation on a surface at room temperature. It is never heated, otherwise crystallization to another form results. The particle size of the hexagonal zinc cadmium sulphide should be smaller than that of the X-ray responsive phosphor, viz. about 5 microns, and the deposit should be thinner, viz. about 10 milligrams per sq. centimeter.

In Fig. 4, there is shown a second embodiment of the invention in which numerals utilized hereinbefore are employed to identify like elements. In this embodiment, electron gun 5 is replaced by a photoemissive layer 30, suitably supported within envelope 2 and maintained at ground potential by a conductive lead 30', and an electroluminescent cell 31 attached mechanically or with an adhesive to the exterior of envelope 2

as illustrated, or supported separate from but near the envelope. Photosensitive material 30 has the property of emitting electrons when irradiated with visible light while electroluminescent cell 31 has the property of emitting visible light when energized by an alternating current source 33. In this manner an electron beam 32 having a desired highly uniform current density is produced and accelerated by the potential upon conductive coating 19.

Photosensitive layer or screen 30 is preferably composed of antimony on which a caesium layer has been deposited by flashing in a vacuum and which, after such deposit, has been heated to a temperature between 150° C. and 210° C. to form a caesium antimony compound (CS<sub>2</sub>Sb; probably a mixture of CS<sub>2</sub>Sb and CS<sub>3</sub>Sb). Other suitable photosensitive surfaces may be produced by flashing caesium on arsenic or bismuth or any mixture of arsenic, antimony or bismuth; heating is also satisfactory. Surfaces produced by flashing other metals of the alkali group, particularly rubidium, or mixtures of these metals on deposits of arsenic, antimony or bismuth or mixtures of these may also be employed with efficacy.

Electroluminescent cell 31 is a light-emitting device made after the manner of a flat plate capacitor, except that one of the plates is made of a transparent conducting material such as tin oxide and the space between the plates is occupied by a thin layer of dielectric material in which a phosphor such as zinc sulphide is suspended. When such a device is energized by alternating current, the phosphor emits light which is visible through the transparent conducting layer. The intensity of the light increases as the voltage and frequency of the alternating current increase. A suitable cell of this nature is disclosed in the United States patent application of Jerome S. Prener, assigned to the assignee of the present invention, filed September 8, 1951, and having Serial No. 245,696.

In both the embodiments illustrated, a magnetic field generated by a solenoidal winding disposed about the exterior of tube envelope 2 may be employed to secure desired axial focusing of the electron beam. Also, it should be denoted that for any level of incident X-ray intensity which, of course, determines the conductance of the photoconductor, the current density of the electron beam should be adjusted for maximum contrast in the final intensified light image.

It is to be particularly observed that the term "mesh" is intended herein to include all equivalent forms of apertured elements capable of performing the function set forth in connection therewith, e. g. apertured plates, screens, sieves, etc.

While the invention has been described by reference to particular embodiments thereof, alternative constructions will readily occur to those skilled in the art. Therefore, it is intended in the appended claims to cover all such equivalent embodiments as may be within the true spirit and scope of the foregoing description.

What I claim as new and desire to secure by Letters Patent of the United States is:

1. An image intensification tube comprising means for generating a defocused electron beam directed along an optical axis; an image conversion means spaced from said beam generating means and traversing said optical axis including an X-ray responsive phosphor for receiving X-ray images and forming corresponding light images, and a photoconductor adjacent said X-

ray responsive phosphor between said electron beam generating means and said X-ray responsive phosphor for receiving electrons from said beam generating means and transforming the light images formed by said X-ray responsive phosphor into reversely corresponding charge images; an apertured electron-permeable element positioned traversing said optical axis between said beam generating means and said photoconductor and having an electron-responsive phosphor deposited on the side thereof opposite said beam generating means whereby electrons in said electron beam may pass through said apertured electron-permeable element without exciting said electron-responsive phosphor, the charge images on said photoconductor being effective to reverse the direction of travel of electrons passing through said apertured electron-permeable element and approaching the portions of the charge images whereby the reversed electrons impinge upon said electron-responsive phosphor to form intensified light images reversely corresponding to the X-ray images formed on said X-ray responsive phosphor.

2. An image intensification tube comprising means for generating a defocused electron beam directed along an optical axis; an image conversion means spaced from said beam generating means and traversing said optical axis including an X-ray responsive phosphor for receiving X-ray images and forming light images corresponding to the X-ray images, a thin transparent conductive element adjacent said X-ray responsive phosphor between said beam generating means and said X-ray responsive phosphor, and a photoconductor contiguous with the surface of said transparent conductive element remote from said X-ray responsive phosphor for receiving and storing electrons from said electron beam, the light images upon said X-ray responsive phosphor being effective to irradiate portions of said photoconductor and discharge electrons therefrom through said transparent conductive element to produce reverse charge images on said photoconductor; a mesh positioned to traverse said electron beam between said beam generating means and said image conversion means; an electron-responsive phosphor deposited on the side of said mesh remote from said beam generating means whereby electrons in said electron beam may pass from said beam generating means through the interstices of said mesh without exciting said electron-responsive phosphor, the charge images on said photoconductor being effective to reverse the direction of travel of electrons passing through said mesh and approaching the portions of the charge images whereby the reversed electrons impinge upon said electron-responsive phosphor to form intensified light images reversely corresponding to the X-ray images formed on said X-ray responsive phosphor.

3. An image intensification tube as in claim 2 in which said beam generating means comprises an electron gun including a thermionically emissive cathode and an accelerating anode.

4. An image intensification tube as in claim 2 in which said beam generating means comprises an electro-luminescent cell for generating visible light and a photoemissive layer adjacent said cell for emitting electrons along said optical axis in response to the visible light emanating from said cell.

5. An image intensification tube comprising means for generating a defocused electron beam

directed along an optical axis; an image conversion means spaced from said beam generating means and traversing said optical axis including an X-ray responsive phosphor for receiving X-ray images and forming light images corresponding to the X-ray images, a thin transparent conductive element adjacent said X-ray responsive phosphor between said beam generating means and said X-ray responsive phosphor, and a photoconductor contiguous with the surface of said transparent conductive element remote from said X-ray responsive phosphor for receiving and storing electrons from said electron beam, the light images upon said X-ray responsive phosphor being effective to irradiate portions of said photoconductor and discharge electrons therefrom through said transparent conductive element to produce reverse charge images on said photoconductor; a mesh positioned to traverse said electron beam between said beam generating means and said image conversion means; an electron-responsive phosphor deposited on the side of said mesh remote from said beam generating means whereby electrons in said electron beam may pass from said beam generating means through the interstices of said mesh without exciting said electron-responsive phosphor, the charge images on said photoconductor being effective to reverse the direction of travel of electrons passing through said mesh and approaching the portions of the charge images whereby the reversed electrons impinge upon said electron-responsive phosphor to form intensified light images reversely corresponding to the X-ray images formed on said X-ray responsive phosphor, and means for observing said intensified light images.

6. An image intensification tube comprising means for generating a defocused electron beam directed along an optical axis; an image conversion means spaced from said beam generating means and traversing said optical axis including an X-ray responsive phosphor for receiving X-ray images and forming light images corresponding to the X-ray images, a thin transparent conductive element adjacent said X-ray responsive phosphor between said beam generating means and said X-ray responsive phosphor, and a photoconductor contiguous with the surface of said transparent conductive element remote from said X-ray responsive phosphor for receiving and storing electrons from said electron beam, the light images upon said X-ray responsive phosphor being effective to irradiate portions of said photoconductor and discharge electrons therefrom through said transparent conductive element to produce reverse charge images on said photoconductor; a mesh positioned to traverse said electron beam between said beam generating means and said image conversion means; electron-optical means adjacent said mesh for causing the electrons in said beam to follow paths approximately parallel to said optical axis; an electron-responsive phosphor deposited on the side of said mesh remote from said beam generating means whereby electrons in said electron beam may pass from said beam generating means through the interstices of said mesh without exciting said electron-responsive phosphor, the charge images on said photoconductor being effective to reverse the direction of travel of electrons passing through said mesh and approaching the portions of the charge images whereby the reversed electrons impinge upon said electron-responsive phosphor to form intensified light images.

images reversely corresponding to the X-ray images formed on said X-ray responsive phosphor.

7. An image intensification tube as in claim 4 in which said electron-optical means comprises a conductive coating along a portion of the interior surface of said tube.

8. An image intensification tube as in claim 4 in which said electron-optical means comprises a conductive coating along a portion of the interior surface of said tube on the side of said mesh adjacent said beam generating means, said conductive coating being connected to said mesh.

9. Image intensification apparatus comprising means for generating a disperse electron beam

15 directed along an optical axis; an image conversion means spaced from said beam generating means and traversing said optical axis including an X-ray responsive phosphor for receiving X-ray images and forming light images corresponding to the X-ray images, a thin transparent conductive element adjacent said X-ray responsive phosphor between said beam generating means and said X-ray responsive phosphor, and a photoconductor contiguous with the surface of said transparent conductive element remote from said X-ray responsive phosphor for receiving and storing electrons from said electron beam, the light images upon said X-ray responsive phosphor being effective to irradiate

20 portions of said photoconductor and discharge electrons therefrom through said transparent conductive element to produce reverse charge images on said photoconductor; a circuit connected to said transparent conductive element for 25 dissipating the discharged electrons from said photoconductor; an electron-permeable mesh positioned to traverse said electron beam between said beam generating means and said image conversion means; an electron-responsive phosphor deposited on the side of said mesh remote from said beam generating means whereby electrons in said electron beam may pass from said beam generating means through the interstices of said mesh without exciting said electron-re-

30 sponsive phosphor, the charge images on said photoconductor being effective to reverse the direction of travel of electrons passing through said mesh and approaching the portions of the charge images whereby the reversed electrons impinge upon said electron-responsive phosphor to form intensified light images reversely corresponding to the X-ray images formed on said X-ray responsive phosphor; and means for viewing said intensified light images.

35 10. Image intensification apparatus comprising an evacuable envelope, means for generating a disperse electron beam within said envelope directed along an optical axis; an image conversion means within said envelope spaced from said beam generating means and traversing said optical axis including an X-ray responsive phosphor for receiving X-ray images and forming light images corresponding to the X-ray images, a thin transparent conductive element adjacent said

40 X-ray responsive phosphor between said beam generating means and said X-ray responsive phosphor, and a photoconductor contiguous with the surface of said transparent conductive element remote from said X-ray responsive phosphor for receiving and storing electrons from said electron beam, the light images upon said X-ray responsive phosphor being effective to irradiate portions of said photoconductor and discharge electrons therefrom through said trans-

45 parent conductive element to produce reverse 50 images reversely corresponding to the X-ray images formed on said X-ray responsive phosphor.

55 11. Image intensification apparatus comprising an evacuable envelope, means for generating a disperse electron beam within said envelope directed along an optical axis; an image conversion means within said envelope spaced from said beam generating means and traversing said optical axis including an X-ray responsive phosphor for receiving X-ray images and forming light images corresponding to the X-ray images, a thin transparent conductive element adjacent said

55 X-ray responsive phosphor between said beam generating means and said X-ray responsive phosphor, and a photoconductor contiguous with the surface of said transparent conductive element remote from said X-ray responsive phosphor for receiving and storing electrons from said electron beam, the light images upon said X-ray responsive phosphor being effective to irradiate portions of said photoconductor and discharge electrons therefrom through said trans-

60 parent conductive element to produce reverse images reversely corresponding to the X-ray images formed on said X-ray responsive phosphor.

## 11

charge images on said photoconductor; a circuit connected through said envelope to said transparent conductive element for dissipating the discharged electrons from said photoconductor; an electron-permeable mesh positioned to traverse said electron beam between said beam generating means and said image conversion means; electron-optical means adjacent said mesh for causing the electrons in said beam to follow paths approximately parallel to said optical axis; an electron-responsive phosphor deposited on the side of said mesh remote from said beam generating means whereby electrons in said electron beam may pass from said beam generating means through the interstices of said mesh without exciting said electron-responsive phosphor, the charge images on said photoconductor being effective to reverse the direction of travel of electrons passing through said mesh and approaching the portions of the charge images whereby the reversed electrons impinge upon said electron-responsive phosphor to form intensified light images reversely corresponding to the X-ray images formed on said X-ray responsive phosphor; and means for viewing said intensified light images from the exterior of said envelope.

11. Image intensification apparatus as in claim 10 in which said beam generating means comprises an electron gun including a thermionically emissive cathode and an accelerating anode.

12. Image intensification apparatus as in claim 10 in which said beam generating means comprises an electro-luminescent cell for generating visible light and a photo-emissive layer adjacent said cell for emitting electrons along said optical

30  
35

## 12

axis in response to the visible light emanating from said cell.

13. Image intensification apparatus as in claim 10 in which said electron-optical means comprises a conductive coating along a portion of the interior surface of said envelope.

14. Image intensification apparatus as in claim 10 in which said electron-optical means comprises a conductive coating along a portion of the interior surface of said envelope on the side of said mesh adjacent said beam generating means, said conductive coating being connected to said mesh and being maintained at a relatively high potential with respect to said beam generating means.

15. Image intensification apparatus as in claim 14 in which said circuit is connected through said envelope to both said transparent conductive element and said photoconductor.

16. Image intensification apparatus as in claim 14 in which said circuit is connected through said envelope to both said transparent conductive element and said photoconductor and includes a source of direct voltage for maintaining a difference of potential between the potential of origination of said electrons and the potential of said photoconductor.

FERD E. WILLIAMS.

## References Cited in the file of this patent

## UNITED STATES PATENTS

| Number    | Name         | Date           |
|-----------|--------------|----------------|
| 2,203,347 | Batchelor    | June 4, 1940   |
| 2,277,246 | McGee et al. | Mar. 24, 1942  |
| 2,523,132 | Mason et al. | Sept. 19, 1950 |
| 2,577,038 | Rose         | Dec. 4, 1951   |